



US005383513A

**United States Patent** [19]

Revankar

[11] **Patent Number:** 5,383,513[45] **Date of Patent:** \* Jan. 24, 1995[54] **HARD FACING CASTING SURFACES WITH WEAR-RESISTANT SHEETS**[75] Inventor: **Gopal S. Revankar**, Moline, Ill.[73] Assignee: **Deere & Company**, Moline, Ill.

[\*] Notice: The portion of the term of this patent subsequent to Dec. 7, 2010 has been disclaimed.

[21] Appl. No.: 53,697

[22] Filed: **Apr. 29, 1993****Related U.S. Application Data**

[63] Continuation-in-part of Ser. No. 822,904, Jan. 21, 1992, Pat. No. 5,267,600.

[51] Int. Cl.<sup>6</sup> ..... B22D 19/14; B22D 19/08[52] U.S. Cl. ..... 164/97; 164/111;  
164/112[58] **Field of Search** ..... 164/97, 98, 100, 103,  
164/111, 112[56] **References Cited****U.S. PATENT DOCUMENTS**

- 1,978,319 10/1934 Mowery ..... 164/112  
 2,874,429 2/1959 Emter et al. ..... 164/111  
 4,119,459 10/1978 Ekemar et al. .....  
 4,254,621 3/1981 Nagumo ..... 164/97  
 4,646,811 3/1987 Morishita ..... 164/9  
 4,875,616 10/1989 Nixdorf ..... 164/97  
 4,955,121 9/1990 Sato et al. ..... 164/98  
 4,972,898 11/1990 Cole ..... 164/98

5,027,878 7/1991 Revankar .  
 5,190,091 3/1993 Revankar .  
 5,190,092 3/1993 Revankar .

**FOREIGN PATENT DOCUMENTS**

- 0297552 1/1989 European Pat. Off. .  
 5125211 7/1976 Japan ..... 164/97  
 0026565 8/1978 Japan ..... 164/97  
 0192671 11/1983 Japan ..... 164/97  
 2074912 11/1981 United Kingdom .  
 1163977 6/1985 U.S.S.R. ..... 164/97

*Primary Examiner*—P. Austin Bradley*Assistant Examiner*—Erik R. Puknys*Attorney, Agent, or Firm*—Burns, Doane, Swecker & Mathis[57] **ABSTRACT**

A method for impregnating a metal product with a hard wear-resistant surface area comprises providing a wear-resistant layer in the form of a sintered sheet having a pattern which facilitates metallurgical bonding with a metal melt and optionally, at least one “pin” integrally attached onto a surface of the sheet. This wear-resistant layer is attached onto the sand core and a metal melt is cast so as to produce the final product. This method can be used to produce a variety of metal products although cast iron is preferred. Moreover, this process can effectively employ any of the hard phases which can be sintered, e.g., tungsten carbide, chromium carbide, and the like.

20 Claims, 3 Drawing Sheets





FIG. 1



FIG. 3



**FIG. 2**



**FIG. 4**



**FIG. 5**

## HARD FACING CASTING SURFACES WITH WEAR-RESISTANT SHEETS

### CROSS-REFERENCE TO RELATED APPLICATION

This application is a continuation-in-part of Ser. No. 07/822,904, filed Jan. 21, 1992 now U.S. Pat. No. 5,267,600 is incorporated herein by reference in its entirety for all purposes.

### BACKGROUND OF THE INVENTION

#### A) Field of the Invention

The present invention relates to a process for the impregnation of a metal product with a surface comprising a hard wear-resistant material.

#### B) Wear-Resistant Surface Layers in Iron

A wide variety of techniques are known for the impregnation of metals, e.g., iron, with a hard wear-resistant surface. Such techniques include flame spray coating and plasma spray coating. However, each of these spray coating techniques suffer from problems associated with the spalling of surface layers during the coating process and during service as well as the particularly large expense associated with the use of this technique.

Cast-in-carbides are also known in which carbide particulates are placed in a mold and molten iron is then cast. See, for example, the discussion within U.S. Pat. No. 4,119,459 to Eckmar et al. It is difficult, however, with such castings to accurately maintain the carbide particles in the desired location and in a regular distribution pattern during casting.

In addition, certain cast-on hard surfacing techniques for use with polystyrene patterns are also known in the art. See, for example, the discussion in Hansen et al., "Application of Cast-On Ferrochrome-Based Hard Surfacing to Polystyrene Pattern Castings," Bureau of Mines Report of Investigations 8942, U.S. Department of the Interior, 1985.

However, this process suffers from problems associated with the low reliability of the bond formed between the wear-resistant layer, e.g., tungsten carbide, and the foam pattern. Also when thick powder layers are used, the iron may not penetrate the layer before the iron solidifies. Due to these reasons, instead of impregnating the iron, the carbide spalls off the product.

The inventor of the present invention has also been involved in inventing other processes in an attempt to more effectively impregnate the surface of a metal, e.g., iron, with hard phases during the casting process. For example, attention is directed toward U.S. Pat. No. 5,027,878 to Revankar et al which relates to the carbide impregnation of cast iron using evaporative pattern castings (EPC) as well as U.S. Pat. Nos. 5,190,091 and 5,190,092, which relate to the impregnation of cast iron and aluminum alloy castings with carbides using sand cores.

However, despite their effectiveness, these methods also have certain drawbacks. For example, the EPC method may involve the installation of special equipment in a conventional foundry. Furthermore, castings produced by this process can suffer from distortion due to the distortion of the plastic foam replicas. On the other hand, the above sand core methods of casting carbides can involve the preparation of carbide spheres which adds to the cost of the process. The cost can be further increased if a substantially flat wear-resistant

surface is desired because in such a case, a surface layer equal in thickness to approximately half the sphere diameter will need to be machined off.

Accordingly, the need still exists for a method of impregnating metal surfaces, and in particular iron surfaces with a hard wear-resistant material which is capable of overcoming the problems associated with known techniques.

### SUMMARY OF THE INVENTION

In one aspect of the present invention, there is disclosed a method for impregnating a metal product with a hard wear-resistant material surface layer.

In another aspect, the present invention relates to a method for impregnating a metal product with a hard wear-resistant surface layer comprising:

(a) providing a wear-resistant material layer in the form of a sintered sheet having a discernable pattern on one surface thereof, which pattern facilitates metallurgical bonding with a metal melt and, optionally, at least one pin integrally attached onto the surface thereof;

(b) attaching the wear-resistant layer to a mold surface; and

(c) casting a metal melt at an effective temperature so as to produce a metal product having a wear-resistant material surface layer which metal is selected so as to metallurgically bond to the wear-resistant layer.

In one embodiment, the effective temperature is less than the melt temperature of the wear-resistant material.

In another embodiment, the wear-resistant layer includes "pins" or "hooks" made from the wear-resistant material and which enhances the "mechanical" attachment of the layer to the casting surface.

In another aspect, the present invention relates to the product produced by this method.

### BRIEF DESCRIPTION OF THE DRAWINGS

FIG. 1 illustrates a sintered carbide sheet containing four carbide "pins" according to the present invention.

FIG. 2 illustrates suitable shapes for the carbide pins which are employed in the present invention.

FIG. 3 is a photograph illustrating a ductile iron casting showing a carbide sheet having a "hook" or "pin" forming an integral part of the sheet.

FIGS. 4 and 5 are photographs illustrating two patterns for wear-resistant surfaces according to the present invention.

### DETAILED DESCRIPTION OF THE PREFERRED EMBODIMENTS

The present invention can be employed for casting virtually any type of metal which is known within the art. However, cast iron, and in particular, ductile or grey iron are preferred. Other examples of suitable metals include non-ferrous alloys and superalloys.

In the present invention, an initial step involves the formation of a sheet comprising a wear-resistant material. As to the choice of the hard wear-resistant material, the present invention can effectively employ any of the hard phases which can be sintered, such as tungsten carbide, chromium carbide, and the like.

Furthermore, this wear-resistant material can include a metallic binder, such as those of the Fe group, preferably Co for use with tungsten carbide, or Ni for chromium carbide, and the like. For example, where ductile

iron is employed as the metal to be cast, particles composing tungsten carbide with 12-17 weight % cobalt is preferred.

The sheet is formed by mixing a powder of the hard wear-resistant material (optionally containing a metallic binder) with a suitable organic binder, for example, a 10% polyvinyl alcohol (PVA) solution, and a suitable plasticizer, for example, 2-ethylhexyl diphenyl phosphate, phosphate ester plasticizer (e.g., KRONITEX 3600 of FMC Corporation) or a mixture of plasticizers so as to form a slip which has appropriate rheological characteristics such that it can be formed into a sheet. In this regard, suitable binders and/or plasticizers include any which can be effectively employed with the particular wear-resistant material.

In this process, fine particles of the wear-resistant material are preferably employed, i.e., -140/200 and finer mesh size.

The outer surface of the sheet is then preferably patterned into a texture which allows for better impregnation of the iron.

It is believed that the bonding of the present invention relates to the diffusion of the molten metal, e.g., iron, into the sheet, e.g., the carbide/cobalt composite. This pattern is, thus, selected so as to facilitate the strength of the metallurgical bond formed between the metal and the wear-resistant material. In this regard, the use of the patterns allowed for a suitable strength bond by surface diffusion to a depth as small as 100 microns.

For example, the pattern contains a "waffle" or a plurality of "ridges" which can effectively react with the molten metal. See, for example, the patterns illustrated in FIGS. 4 and 5.

Furthermore, it is preferred that these ridges are discernible, i.e., retain a substantial portion of their shape, after casting of the metal melt. See, for example, FIG. 3.

This pattern can also be selected so as to prevent the lateral movement of the sheet from the component surface during use, i.e., to allow it to resist any shear force that may be applied tangentially to the sheet surface.

Moreover, this pattern can be formed by any suitable means, for example, by pressing a die with the required pattern onto the surface of the sheet while the sheet is still green and in the plastic state.

The same wear-resistant material/organic binder/plasticizer mixture employed in producing the sheet is also preferably employed in forming the optional "pins" or "hooks" which can be attached to the sheets. The shape of these "pins" or "hooks" is any shape which allows it to "mechanically" hold the wear-resistant material sheet onto the casting surface. Two examples of suitable pin shapes are illustrated by FIG. 2. Other pin shapes can include, e.g., flat "sheets" of carbides, also having a waffle surface texture.

These pins are cast separately and then dried, e.g., in an oven at, e.g., 100° C. so as to become a "rigid" solid. These pins are planted onto the sheet and in particular, onto the side of the sheet containing the pattern so as to form the wear-resistant layer, when the sheet is still green and soft. See, for example, the arrangement illustrated in FIG. 1.

The number of pins which are optionally attached to the sheet are those which aid in overcoming the force of separation that may be applied to the sheet surface. For example, in the embodiment illustrated by FIG. 1, four

hooks are employed although, the number can vary from, e.g., 1-8 pins.

These pins can be attached after they are dried, or, they can be presintered and then attached onto the sheets. In either technique, they become an integral part of the sheets when the sheets themselves are dried along with the attached pins. These sheets are then heated at low temperatures e.g., 320°-340° C. to partially remove organic binder and plasticizer.

The sintering of the "green" sheet after its drying occurs under suitable conditions to allow the sheet and the pins to become fully dense and a single body. Suitable sintering conditions are recognized in the art and include, for example, that occurring in a vacuum at 1450°-1475° C. for 50-75 minutes.

Because the composition of the pin is preferably identical to that of the sheet, the sintered sheet with the hooks attached is effectively stress-free when cooled to room temperature from the sintering temperature and thus, the pins form an integral part of the sheets subsequent to sintering. See, for example, the cross-section illustrated in FIG. 3.

Though the above described method uses binder and plasticizer to form sheets (and the optional pins) there may be other methods which may not use these organic additives. Thus for example, the carbide powder with a suitable proportion of metallic binder may be directly pressed into a sheet with a flat pin or without any pin in a cold die press. Such sheets may then be sintered following the same procedure as for making carbide sheets using organic binders and plasticizers except, of course, that the step for removal of binder and plasticizer by heating at lower temperatures is unnecessary.

The sintered wear-resistant layer is then attached onto a suitable mold surface, e.g., a sand core by means which are recognized within the art. For example, in one embodiment, a high temperature adhesive is employed and the layer is then heated in, e.g., an oven at 100° C. so as to drive moisture from the adhesive and cure it.

By high temperature, it is meant that the adhesive has a melting point higher than the metal pouring temperature. Any suitable adhesive can be employed within the present invention with high temperature inorganic adhesive being preferred.

In the preferred embodiment employing ductile iron as the metal, the binder comprises a high temperature ceramic adhesive, AREMCO's Ceramabond 569, which is a proprietary high temperature binder that includes oxides of aluminum, silicon and potassium, as a colloidal suspension in water and which has a maximum use temperature of about 1650° C. (Ceramabond is a trademark of AREMCO Products, Inc.).

At this point, the liquid metal is cast around the hard wear-resistant layer using any of the casting techniques traditionally employed in the art, e.g., gravity feed casting, squeeze casting, vacuum casting or the like. However, due to the ease of use, the gravity feed of metal is preferred.

The particular metal employed is not critical to the present invention. However, it should be noted that when the metal which is employed is effective in forming a metallurgical bond with the wear-resistant material, e.g., iron with a carbide sheet, no pins are needed in the wear-resistant layer. However, if the molten metal does not form an effective metallurgical bond with the wear-resistant material, e.g., when aluminum or an alloy

thereof is employed with carbide type wear-resistant layer, pin(s) should be employed in wear-resistant layer.

The pouring temperature of the metal is not particularly critical to the invention but, for best results, is preferably done within the range 1350°–1450° C. For example, it can be selected so as to be lower than the melt temperatures of the sheet. In one embodiment, a temperature of 1390°–1400° C. is employed which is lower than the melt temperature of either the tungsten carbide, (i.e., greater than 2700°C.) and the cobalt (i.e., 1495°C.).

An exemplary ductile iron casting with tungsten carbide impregnation is illustrated in FIG. 3.

The method according to the present invention can be used to produce metal products which have a wide variety of applications.

Moreover, the process of the present invention can provide these products at a greatly reduced cost when compared with prior art systems. In particular, the surface modification can be effectively accomplished during the casting process without requiring any subsequent brazing or welding or prior substrate machining and without requiring additional casting facilities such as that associated with the EPC system. In fact, this process can be easily adapted to existing sand casting foundry practices.

In order to further illustrate the present invention and the advantages associated therewith, the following specific example is given, it being understood that same is intended only as illustrated and in no wise limitative.

## EXAMPLES

### Example 1

Fine tungsten carbide/12–17% cobalt powder (–140/200 or finer mesh size) is mixed with a suitable binder such as a 10% aqueous polyvinyl alcohol solution and a suitable plasticizer (2-ethylhexyl diphenyl phosphate or KRONITEX 3600 of FMC Corporation) or a mixture of plasticizers to form a slip with appropriate rheological characteristics so it can be cast or rolled into a sheet. The sheet surface is patterned into a "waffle" texture such as that illustrated by FIG. 4, before the sheets become rigid through drying or curing.

The green carbide sheets are heated at 100° C. so as to become rigid. They are then heated to 340° C. to remove organic binders and plasticizers and are then sintered in vacuum at 1460° C. for 60 minutes when the sheets become fully dense. See FIG. 3.

The sintered carbide sheet is then attached to a sand core using Aremco's Ceramabond 569 and the core/sheet is heated in an oven at 100° C. to drive out the moisture from the binder and cure it. In the alternative, it may be dried at room temperature provided sufficiently long curing time is allowed.

Cast iron is cast around the sheet using the conventional casting practice such that, on metal solidification, the carbide sheet is firmly attached to the casting surface.

### Example 2

Using the same carbide/binder/plasticizer mixture, pins of a suitable shape (see FIG. 2) are cast separately and are dried in an oven at 100° C. when they become rigid solids. These pins are planted into the green carbide sheets on the waffle pattern side of the sheet as shown in FIG. 1, while the sheets are still plastic, i.e., before the binder resin hardens.

The green carbide sheet is then treated as in Example 1.

While the invention has been described in terms of various preferred embodiments, the skilled artisan will appreciate the various modifications, substitutions, omissions, and changes which may be made without departing from the spirit thereof. Accordingly, it is intended that the scope of the present invention be defined solely by the scope of the following claims including equivalents thereof.

### What is claimed:

1. A method for impregnating a metal product with a hard wear-resistant surface layer comprising:

(a) providing a wear-resistant layer in the form of a sintered sheet having a pattern comprising a plurality of ridges on one surface thereof, which pattern facilitates the metallurgical bonding strength between the sheet and a metal melt;

(b) attaching the wear-resistant layer to a mold surface; and

(c) casting the metal melt at an effective temperature to produce a metal product having a wear-resistant material surface layer which metal is selected so as to metallurgically bond with the wear-resistant layer.

2. The method according to claim 1 where the effective temperature is less than the melt temperature of wear-resistant material.

3. The method according to claim 1 wherein the pattern is a discernable pattern.

4. The method according to claim 1 wherein the mold surface is a sand core.

5. The method according to claim 4 wherein the layer is attached to the sand core using a high temperature adhesive.

6. The method according to claim 5 wherein the high temperature adhesive comprises a high temperature ceramic adhesive.

7. The method according to claim 1 wherein the metal is iron.

8. The method according to claim 7 wherein the iron is ductile iron.

9. The method according to claim 1 wherein the hard wear-resistant material comprises tungsten carbide with a metallic binder.

10. The method according to claim 9 wherein the tungsten carbide includes 12–17 weight percent cobalt.

11. The method according to claim 1 wherein the sheet is formed from a mixture of a powder of the wear-resistant material, an organic binder, and at least one plasticizer.

12. The method according to claim 11 further including at least one pin which is made from the same mixture as the sheet.

13. The method according to claim 1 wherein the mold surface is a sand core.

the pattern comprises a waffle pattern; and the sheet is formed from a mixture of a powder of the wear-resistant material, and organic binder, and at least one plasticizer.

14. The method according to claim 13 where iron is cast.

15. The method according to claim 1 wherein unsintered pins are attached to the sheet and the sheet is then sintered.

16. The method according to claim 1 wherein sintered pins are attached to the sheet and the sheet is then sintered.

17. The method according to claim 1 wherein the sheet has at least one pin integrally attached onto the one surface thereof.

18. The method according to claim 17 wherein the effective temperature is less than the melt temperature of the wear-resistant material.

19. The method according to claim 17 wherein the

mold surface is a sand core, the pattern comprises a waffle pattern; and

a sheet and pin(s) are formed from a mixture of a powder of the wear-resistant material, an organic binder, and at least one plasticizer.

20. The method according to claim 19 where iron is cast.

\* \* \* \* \*